

## UNITED STATES PATENT OFFICE

2,593,173

## PROCESS OF REFINING CHEMICAL PULP

Turma Norta and Yrjö Sivola, Imatra, Finland,  
assignors to Enso-Gutzeit Osakeyhtiö, Helsinki,  
Finland, a corporation of the Community of  
Jaaski in the Republic of Finland

No Drawing. Application July 31, 1947, Serial  
No. 765,248. In Sweden October 30, 1943

Section 1, Public Law 690, August 8, 1946  
Patent expires October 30, 1963

5 Claims. (Cl. 8—105)

## 1

When refining chemical pulp according to chemical methods variations in lignin content and viscosity often cause great difficulties in normal refining processes wherefore, generally, very even quality is demanded of chemical pulp intended for some special purpose. One of the properties required of e. g. viscose pulp is that it has a specified viscosity and here no greater variations than 1 cp. are as a rule permissible. In order to reduce and smooth out viscosity the preparation of such viscose pulp has resorted to rigorous hypochlorite treatment. The violence of this treatment is evidenced inter alia by a drop in the percentage amount of the most valuable ingredient of chemical pulp, i. e. alpha cellulose, and by the rise of the copper number, which designates the amount oxycellulose.

On investigating methods for obviation of the above mentioned defects it was found that if washed, defibred and strained chemical pulp was chlorinated and subsequently heated as a 1-15 per cent aqueous suspension to a temperature somewhat exceeding that of a room and kept at this temperature a specified period of time dependent on the quality of chemical pulp under treatment, ranging in practise from 10-200 min., the cellulose molecules break up, partly through the agency of acid substances created during chlorination, thus causing a drop in viscosity. As already mentioned, heating must be carried out at a temperature exceeding that of a room, preferably at 40° C.; however it is not advisable to exceed 100° C. because of practical and economical reasons. The heating of chemical pulp can also be applied subsequently to partial or complete washing, but in this case care must be taken to adjust, e. g. by means of adding acids, the pH-value of the chemical pulp suspension below 5. The drop in the pH-value can also be accomplished by introducing chlorine into the suspension, thus simultaneously removing the lignin residues from the chemical pulp. In view of the result it makes no difference whether "hydrolysis" is carried out in apparatus operating periodically or continuously. The advantages, achieved by the process hereinabove described as compared with the hypochlorite treatment generally used at the moment, are that inter alia the alpha content of the chemical pulp increases, the pentosan content decreases and the copper number drops.

What we claim is:

1. A process of making refined chemical pulp

## 2

comprising, selecting washed, defibred and strained chemical pulp, chlorinating such pulp at room temperature, forming such pulp into a 1-15% aqueous suspension partially washed with water, and heating such pulp at a temperature above room temperature but not over 100° C. for a period of time of about 10 to 200 minutes at a pH value lower than 5.

2. A process as defined in claim 1 and including adding acid to the partially washed chemical pulp after chlorination in sufficient amount to lower the pH value under 5.

3. A process as defined in claim 1 and including introducing chlorine into the pulp while the heating is taking place to lower the pH value under 5.

4. A process of making refined chemical pulp comprising, selecting washed, defibred and strained chemical pulp, chlorinating such pulp at room temperature, then heating such pulp at a temperature above that of room temperature but below 100° C., and continuing that heating for a period of time at about 10 to 200 minutes at a pH value lower than 5.

5. A process of making refined chemical pulp comprising, selecting washed, defibred and strained chemical pulp, chlorinating such pulp at room temperature, subsequently heating such pulp as a 1-15% aqueous suspension at a temperature of approximately 40° C. and continuing such heating for a period of time of from 10 to 200 minutes at a pH value lower than 5.

TURMA NORTA.  
YRJÖ SIVOLA.

## 35

## REFERENCES CITED

The following references are of record in the file of this patent:

## UNITED STATES PATENTS

| 40 | Number    | Name    | Date          |
|----|-----------|---------|---------------|
|    | 1,705,897 | Bradley | Mar. 19, 1929 |
|    | 1,941,154 | Richter | Dec. 26, 1933 |
|    | 1,967,347 | Bayerl  | July 24, 1934 |
| 45 | 2,065,395 | Richter | Dec. 22, 1936 |
|    | 2,070,893 | Glass   | Feb. 16, 1937 |
|    | 2,159,376 | Freeman | May 23, 1939  |
|    | 2,198,706 | Sheldon | Apr. 30, 1940 |

## OTHER REFERENCES

50 Cellulose and its Derivatives, by Ott, published by Interscience Publishers, Inc., N. Y., N. Y., 1943, pp. 588-589, 598, 599, and 603.